

Patented Oct. 4, 1927.

1,644,360

# UNITED STATES PATENT OFFICE.

BENJAMIN TALBOT, OF NORTHLERTON, ENGLAND, ASSIGNOR TO TALBOT NON-CORROSIVE LININGS COMPANY, OF PHILADELPHIA, PENNSYLVANIA, A CORPORATION OF DELAWARE.

## WATER PIPE AND METHOD OF MAKING THE SAME.

No Drawing. Application filed July 5, 1924, Serial No. 724,537, and in Great Britain July 14, 1923.

It is an object of this invention to construct steel or iron water pipes which shall be comparatively light in weight.

Such pipes as at present constructed have to be made of a material considerably heavier than is required merely for withstanding the internal pressure to which they are subjected in use, because they are liable to become weakened by corrosion. This liability could be minimized by coating the pipe internally or externally or both, as may be necessary, with a protective material such as cement, asphalt, concrete or pitch; but this is difficult because of the feeble adhesion between any of these materials and an iron or steel surface. It is an object of my invention to improve this adhesion; the methods of doing so which have been applied to pipes of small diameter, such as condenser tubes, namely by roughening the surface or applying a wire gauze wrapping before the coating operation, are inapplicable to large diameter water pipes.

My invention consists in rolling into pipe form a plate of steel or iron on one or both faces of which there has been produced a serrated or chequered pattern by rolling or pressing the plate in the course of manufacture by a patterned roller or press in known manner; this pipe form becomes a pipe when the edges of the plate are welded together in known manner.

My invention further consists in lining or coating or both lining and coating the finished pipe with a protective material of the kind hereinbefore named.

A diagonal or chequered pattern on the plate is very useful; however, other designs are also satisfactory, such as serrations or ridges in parallel or wavy lines, running either longitudinally or transversely in the pipe to be formed.

Pipes protected from rusting by coverings of the kind in question can be made of lighter material than is safe for uncovered pipes subject to rusting; there is a limit to this diminution of weight, however, because the stiffness of the pipe is impaired as the weight is diminished. The pattern provided according to my invention lends sufficient stiffness to metal of a weight which could not well be used if the metal had a plane surface.

Cylindrical corrugated sheet metal reinforcement in pipes made of concrete or bitu-

minous material is well-known; my invention is in no way concerned with pipes made of such reinforced material.

Having thus fully described the nature of the said invention and the best means I know of carrying the same into practical effect, I claim:

1. A water pipe, light in weight, consisting of a plate of steel or iron having a well defined pattern impressed thereon and which is rolled into pipe form and welded and has a coating of material applied to the patterned surface to protect the metal from rust.

2. A water pipe, light in weight, consisting of a plate of steel or iron having a well defined pattern impressed thereon and which is rolled into pipe form and welded and has a lining of material applied to the patterned surface to protect the metal from rust.

3. A water pipe, light in weight, consisting of a plate of steel or iron having a well defined pattern impressed thereon and which is rolled into pipe form and welded and has a coating and lining of material applied to the patterned surface to protect the metal from rust.

4. A process for the manufacture of water pipes light in weight, which process consists in producing a well defined pattern on a plate of steel or iron, rolling the plate into pipe form, welding the edges and coating the patterned surface with a material adapted to protect metal from rust.

5. A process for the manufacture of water pipes light in weight, which process consists in producing a well defined pattern on a plate of steel or iron, rolling the plate into pipe form, welding the edges and lining the patterned surface with a material adapted to protect the metal from rust.

6. A process for the manufacture of water pipes light in weight, which process consists in producing a well defined pattern on a plate of steel or iron, rolling the plate into pipe form, welding the edges and lining and coating the patterned surface of the pipe with a material adapted to protect metal from rust.

7. A process for the manufacture of water pipes light in weight, which process comprises the step of rolling into pipe form a plate of steel or iron having a well defined pattern on a surface thereof, welding the

edges and coating the patterned surface with a protecting material.

8. A process for the manufacture of pipes which consists in rolling up a sheet of metal having a well defined pattern impressed on the surface thereof and applying to such impressed surface a protective covering, said covering being keyed to said sheet by said patterned surface.

9. The process which consists in rolling a well defined pattern upon the surfaces of a hot iron or steel plate and covering the patterned surfaces with a protective coating keyed to said plate by such patterned surface.

In testimony whereof I have signed my name to this specification.

BENJAMIN TALBOT.